

No. 818,300.

PATENTED APR. 17, 1906.

W. D. SARGENT.

PROCESS FOR MAKING BRAKE SHOES.

APPLICATION FILED NOV. 4, 1903.

2 SHEETS—SHEET 1.

Fig. 1



Fig. 2



Fig. 3



Fig. 4



Fig. 5



Fig. 6



Inventor,

William D. Sargent,

Witnesses;

Edward D. Burney  
Oscar Steinemagel

By Paul Symestrodt

Attorney

No. 818,300.

PATENTED APR. 17, 1906.

W. D. SARGENT.  
PROCESS FOR MAKING BRAKE SHOES.  
APPLICATION FILED NOV. 4, 1903.

2 SHEETS—SHEET 2.

Fig. 7



Fig. 8



Fig. 9



Fig. 10



Fig. 11



Fig. 12



Witnesses;

Edward C. Burns  
Paul Carpenter

By Paul Symmestredt

Attorney

Inventor,  
William D. Sargent,

# UNITED STATES PATENT OFFICE.

WILLIAM DURHAM SARGENT, OF NEW YORK, N. Y., ASSIGNOR TO AMERICAN BRAKE SHOE & FOUNDRY COMPANY, OF NEW YORK, N. Y., A CORPORATION OF NEW JERSEY.

## PROCESS FOR MAKING BRAKE-SHOES.

No. 818,300.

Specification of Letters Patent.

Patented April 17, 1906.

Application filed November 4, 1903. Serial No. 179,831.

*To all whom it may concern:*

Be it known that I, WILLIAM DURHAM SARGENT, a citizen of the United States, residing at New York, in the State of New York, have invented a certain new and useful Process for Making Brake-Shoes, of which the following is a specification.

My invention relates to the wearing blocks used upon the brakes of railway cars and the like, and particularly to the method of making such brake blocks or shoes. The objects of the invention are, to make a composite metal shoe, combining cheaply the strength and wearing qualities of soft iron with the resistance and hardness of cast iron, and to conveniently make such a composite shoe by filling in a supporting shell with the two mixed metals; to provide a method by which a regulable and certain quantity of malleable metal may be inserted in a cast shoe; to provide a process by which malleable steel filaments may be inserted into a brake shoe without melting or destroying their quality, and to provide for even distribution of the various kinds of metal in the wearing surface of the shoe; to provide for chilling the portions of the shoe forming the filling thereof; to provide a cast brake shoe having a malleable metal filling firmly bound to a malleable metal backing, and to generally cheapen and simplify the method of making brake shoes, and improve the structure of the same.

The above objects, together with other advantages which will hereinafter appear, I attain by means of the procedure described herein and illustrated in preferred form in the accompanying drawings, wherein—

Figure 1 is a plan view of the steel back and the position of the metal of the cast shell indicated in dotted lines;

Figure 2 is a central longitudinal section of the back and the shell cast thereon, previous to putting in the filling;

Figure 3 is an under plan view of the shell and filling before the pouring in of the hard cast metal, showing the preferred arrangement of the expanded metal filaments;

Figure 4 is a longitudinal section of the complete shoe showing the cast shell and backing, the filling of malleable metal layers and hard cast metal therein;

Figure 5 is a cross section of the back and shell, taken on line (5) of Figure 2;

Figure 6 is a cross section of the shell filled with the expanded metal, taken on the line (6) of Figure 3.

Figure 7 is a cross section showing a modification in which the shell is made entirely of cast iron and the filling held therein by forming the opening in the back of the shell in a dove-tailed shape as shown;

Figure 8 is a similar central cross section of another modification, in which the attaching lug is made partly of a metallic strap instead of casting said lug;

Figure 9 is a central cross section and half perspective of a form of shoe for use on engine drivers and other places where the shoe and head are made in one piece, and showing the filling attached thereto by an opening or set of openings made of a dove-tailed form to retain the filling;

Figure 10 is an under plan view of a flange brake shoe made for use on drivers, in which the throat of the flange is left open, the shell being entirely cast; and

Figures 11 and 12 are cross sectional views, taken respectively on lines (11) and (12) in Figure 10.

In Figures 1 to 6, I have shown the form of shoe which I prefer, as being strengthened by the steel back; but the broader embodiment of my invention is illustrated by Figure 7, in which the shell is entirely of cast iron and the filling is attached thereto by means of the metal extending through the dove-tailed openings in the back, as will be understood.

The many advantages of having a brake shoe made of composite material including both the hard resisting qualities of cast iron and the drag or superior frictional qualities of soft iron or steel, are well known to the railway trade. In making such shoes, difficulty has been experienced in combining them properly together and with the proper strength and proper connection with the backing of the shoe; and it has also been difficult to make such shoes in such form that the wearing face of the shoe presents uniformly on the wearing face the alternations of hard and soft metal desired. In order to meet the many requirements of a superior brake shoe

in these respects, I first cast an inclosing shell which has walls merely thick enough to hold the parts together and which may be provided with an integral lug for attaching the key and also with seating lugs for the brake head. This shell may be made of various forms and the filling may be attached to the backing either by simply pouring through the cast perforations as illustrated in Figure 7, or, as in the preferred form, as follows:

I may use a steel backing to strengthen the shoe, and in such case I prefer the form of back 7 as shown in Figure 1, having the openings (9) and the cut-out portion (8) near the center to accommodate the metal to hold the attaching lug and the shell together. Placing such a steel back in a mold, I cast around it the shell 10 which will ordinarily be say 5/16th of an inch thick so that it surrounds all the edges of the steel back and forms the key lug and the lugs 12 passing over the part 16. The openings (9) are not filled, and the back and front parts of the steel back are left uncovered, as will be seen from Figure 2. The lug 11 can be either a cast lug, as here shown, or a reinforced or malleable iron lug 11<sup>a</sup> as in Figure 8, if desired. For making this shell portion, I prefer to use a superior quality of soft and tough gray iron.

This cast shell and back, being thus attached together as above described, the walls of the shell and other parts are carefully cleaned, whereupon I pack some form of malleable metal, such as the expanded steel strips illustrated in Figures 3 and 6, in the open space within the shell, preferably placing them alternating in direction as is shown in Figure 3. These may be cut of proper dimensions and placed in the face in whatever proportions are desired and packed as densely as desired. The shell with the expanded metal filaments therein is then placed face down upon a form of sand or iron as may be desired, and the interstices between the filaments of soft metal are filled by pouring in the molten hard cast metal through the openings (9) in the back, thoroughly and completely filling all the space between the malleable metal filaments and flush with the outer edges of the shell, and extending through the openings in the back, forming the necks 15, which may when desired, be slightly lapped over the edges in order to secure a better hold thereon. For this filling I prefer to use a very hard cast iron, for the reasons above set forth.

In the simpler form of the shell as shown in Figure 7, it will be understood, of course, that the procedure is just the same. The openings in the back of the shell 10 are formed narrower toward the front of the shoe than in the rear in order that the neck of the filling, 15<sup>a</sup>, projecting therethrough, will have

a firm hold upon the back even when the filling is worn entirely down. The same procedure also is carried out in the other forms of shoes shown, it being understood that the combined brake head and shoe illustrated in Figure 9 is provided with the projecting dove-tail necks 15<sup>b</sup> extending through proper openings in the back, these openings being of any desired form or number.

It will be observed that this process is particularly advantageous in the making of the form of shoe illustrated in Figures 10, 11, and 12, which is used upon heavy drivers and is so formed that the throat or open space (18) comes upon that part of the wheel which is the most worn upon the rail in running. The filling 14 is attached to the shell 10<sup>b</sup> as before by projecting the neck 15<sup>b</sup> through any number and form of openings in the back of the shell 10<sup>b</sup>, the space (18) being provided in the filling.

It will be observed that by this method of procedure in the pouring of the hard cast metal into the open space and covering the expanded metal, the heat of the cast metal is taken up very largely by the cold side walls of the shell and therefore the molten iron does not destroy the quality of the strands of expanded steel. The filaments of steel are preserved intact throughout the shoe and this greatly adds to the strength of the shoe. The filling is made more dense by this chilling and practically the entire wearing face of the shoe is thus constituted of a combination of dense hard iron, well suited to give durability and hardness, mixed with ductile steel which contributes to superior frictional qualities as well as strength. This combination of metal is firmly locked together and to the steel back, since it will be observed that the filling or briquet portion cast inside, has a hold on the inner edges of the openings of the steel back, while the metal of the sides has an equally firm hold upon the outside edges of the steel back. Thus the two essential cast parts are thoroughly anchored together and to the steel back and the result is a shoe which can hardly be broken apart as it wears down, and the expanded metal presents its superior wearing surface clear through to the extreme back of the shoe, so that the quality of metal exposed to wear is as effective at the end of the life of the shoe as at the beginning. By the thorough distribution of the hard and brittle gray cast iron filling with the malleable steel, they are so placed that they cannot fall out, and at the same time the heat does not destroy the qualities of the malleable filaments, during casting. When the shoe is completely worn out, it will be seen that the parts may be easily broken off and the steel back may be used over again.

Various other advantages of the process and of the form of shoe shown will readily oc-

cur to those familiar with the use of brake shoes.

Having thus described my invention and illustrated its use, what I claim as new, and 5 desire to secure by Letters Patent, is the following:

1. The process of making brake shoes which consists in providing a cast shell of proper form having dove-tailed' openings therein, 10 placing filaments of malleable metal in said shell and pouring in molten metal to fill the interstices between the malleable filaments, extending said filling through the openings to bind the shell and filling together.

15 2. The process of making filled brake shoes which consists in providing a cold shell of iron, partly filling the same with malleable metal pieces, and then pouring in a final filling of molten hard cast metal, whereby the 20 cast filling is chilled in pouring, substantially as and for the purpose described.

25 3. The process of making brake shoes which consists in casting a circumferential shell of cast iron around a steel backing, filling the space in said shell with malleable filaments and filling the interstices between said filaments with cast iron, substantially as described.

30 4. The process of making brake shoes which consists in casting a shell upon the outside edges of a steel back, filling the space formed by the shell and back with filaments of malle-

able iron in skeleton form, and then pouring into the interstices between said filaments a filling of hard cast iron, substantially as described. 35

5. The process of making brake shoes which consists in providing a steel backing having perforations therein, casting thereon a circumferentially arranged shell so as to engage 40 the outer edges of the back, then filling the space in said shell with filaments of malleable steel and filling the interstices between said filaments with molten cast iron, extending the same through the said openings in the 45 steel back, whereby both the shell and the filling of cast metal have a hold upon the edges of said steel back.

6. The process of making brake shoes which consists in providing a cold shell of cast iron 50 in the form of a complete box except for one open side, partly filling the space therein with filaments of malleable metal and then pouring in molten cast iron to fill the interstices between the filaments of malleable 55 metal.

In testimony whereof I have hereunder signed my name in the presence of the two subscribed witnesses.

WILLIAM DURHAM SARGENT.

Witnesses:

M. B. JUSTICE,  
WILLIAM CONOVER.